

June 9, 1942.

J. U. MANN

2,285,526

METHOD FOR PRODUCING CAVITIED RUBBER SHEETING

Filed May 13, 1939

Fig. 1.



Fig. 2.



Fig. 3.



INVENTOR  
JAMES U. MANN  
BY  
Goulding & Bradley  
ATTORNEYS

## UNITED STATES PATENT OFFICE

2,285,526

METHOD FOR PRODUCING CAVITIED  
RUBBER SHEETING

James U. Mann, Arlington, N. J., assignor to  
United States Rubber Company, New York,  
N. Y., a corporation of New Jersey

Application May 13, 1939, Serial No. 273,470

4 Claims. (Cl. 154—2)

This invention relates to methods of producing cavitated rubber sheet material and more particularly to methods of making rubber sheet material having a desired number and arrangement and dimensions of pits or cavities in the surface thereof. This invention is especially advantageous in making any number of replicas of a master cavitated deposition backing or blanket in which the size and arrangement of pits or cavities in each replica are identical with all the others.

According to United States Letters Patent No. 2,032,942, a latex composition is spread onto an air impermeable deposition backing or blanket having cavities or pits in its uppermost surface so as to entrap air within the cavities or pits of the deposition blanket. By the application of heat to the blanket, the thus entrapped air is caused to expand and force its way through the wet latex coating, while at the same time the latex coating is caused to dry or gel so as to render permanent the perforations in the spread film of latex composition. These spreading and heating operations may be repeated until the desired total thickness of perforate rubber sheet has been built up. After the final drying, the perforate rubber sheet is stripped from the blanket and then vulcanized.

While various deposition blankets and methods of making them are described in the above cited patent, the preferred backing is made by coating a woven fabric, such as "4.75 cotton sheeting," with rubber latex in such a manner that the meshes of the fabric are closed on one side of the fabric and are open on the other side, and the individual interstices are also sealed off, each from the other, by the coating of the threads to provide a multitude of pockets opening on the deposition surface of the fabric. A deposition blanket so made has proven satisfactory for making a limited quantity of rubber films or sheets, but upon its wearing out or being defaced the blanket must be replaced by another blanket prepared from another and different piece of fabric. As a consequence it is difficult to prepare a replacement blanket which is identical with the previous one. Furthermore, the described preparation of such blankets is a difficult process, entailing a great deal of care to avoid the preparation of imperfect blankets which must, of course, be discarded.

The present invention provides a method of manufacturing, at relatively low cost, replica deposition blankets which reproduce faithfully the number and arrangement of the pits pres-

ent in the surface of a master deposition blanket which may have been made according to the process described in the above previously cited patent, or by any other suitable process. Any desired number of identically cavitated deposition backings may be produced without the disadvantages and difficulties mentioned. In practicing the invention, a cavitated deposition surface is spread with a film of latex composition, and the latex film thereby deposited is at least partially dried or gelled and concurrently therewith is pierced with a plurality of fluid jets to form permanent perforations therein. A perforate rubber sheet of the desired thickness may be built up by carrying out the above operations the requisite number of times. On the upper surface of this sheet, one or more films of latex composition are then spread so as to bridge and seal off the perforations formed in the lower strata, and this final film (or films) is dried to form a fluid-impermeable continuous sealing film or layer. A sheet of woven fabric or other equivalent inextensible reinforcing material may then be adhered to the sealing film or films either by rolling the fabric down into a wet film of freshly spread latex or rubber cement or by passing the fabric through a bank of latex and under either a doctor blade or a helically grooved cylindrical spreader bar. Other suitable methods of 10 doubling a fabric to a spread sheet of latex rubber may be used conveniently. After the fabric reinforcement has been adhered to the deposition surface one or more additional films of latex rubber may, if desired, be spread thereon and 15 dried to complete the production of an inextensible cavitated sheet. The cavitated sheet may then be removed from the deposition surface upon which it was formed and vulcanized, and the cavitated surface thereof may be treated, as by 20 chlorination or oxidation, to render latex subsequently deposited thereon easily removable 25 therefrom after it has dried or gelled. The resultant cavitated rubber sheet provides an initial master deposition blanket for the production of 30 others identical to it, and the procedure may be 35 repeated as many times as desired, so that the 40 cavities in each rubber sheet deposited thereon 45 will be substantially identical in size and arrangement to those in every other perforate sheet 50 formed therefrom.

By the present invention the possibility of error in reproducing replica blankets identical with the originals is reduced to a minimum. After the perforate plies of the blanket have been produced, and the imperforate ply has been depos-

ited thereon, it may readily be determined merely by inspection whether the imperforate plies have succeeded in sealing off all the perforations in the outermost perforate ply. In the manufacture of cavitated deposition blankets heretofore described, one of the causes of difficulty has been the failure of the treatment of the fabric to satisfactorily seal one opening of each perforation. This previous cause of failure may obviously be eliminated by the present procedure. Another distinct advantage in producing cavitated deposition blankets according to this invention lies in the fact that the entire deposition blanket is built up in a continuous series of operations without the necessity of removing the perforate sheet material from the backing and thereby subjecting it to folding or stretching. The application of an inextensible ply of reinforcing material reduces the possibility of distortion during removal.

The drawing illustrates diagrammatically, on a greatly enlarged scale, a series of steps in the production of identically cavitated rubber sheets according to the present invention, in which:

Fig. 1 is a greatly enlarged cross-sectional view of a master cavitated sheet produced according to the invention on a conventional deposition backing;

Fig. 2 is a greatly enlarged cross-sectional view of a replica cavitated sheet produced from the master; and

Fig. 3 is a greatly enlarged cross-sectional view showing partial removal of the sheet formed in Fig. 2 from the backing on which it is produced.

Referring to the drawing, Fig. 1 shows the formation of a cavitated rubber sheet on a conventional backing 1 comprising woven threads 2 individually impregnated and/or coated with a rubber film 3 and secured to a rubber backing layer 4. On the backing 1 a similar master or backing 5 may be produced as follows: A film or layer 6 of latex is spread onto the backing 1 to entrap air in the pits or cavities between the threads 2, and the backing 1 and film 6 are heated to expand the thus entrapped air sufficiently to form perforations 7 while at the same time the rubber in the film 6 is caused to gel or dry. This process is repeated until a perforate rubber layer 8 of the desired thickness is built up and dried. Before or after completion of the drying of the layer 8, the upper surface 9 thereof is coated with one or more films 10 which may be of the same latex composition as that in the layer 8. This final film (or films) is dried under conditions which do not effect piercing of the rubber covering over perforations 7. For example, the drying or gelling of the film 10 may be accomplished at room temperature without the application of sufficient heat to appreciably expand the entrapped air. The film 10 provides a fluid-impervious and continuous rubber seal which closes off the perforations. A reinforcing or stiffening base ply 11 comprising, for example, one or more fabric layers 12 bonded with rubber, may be secured to the outer surface of the backing 5. After drying the replica blanket 5 may be stripped from the deposition blanket 1 and vulcanized. This vulcanized surface of the initial layer 6 may be halogenated and hardened by treatment with, for example, a 7½% solution of sulphur chloride in carbon tetrachloride, followed by a treatment with a 2 to 3% solution of bromine, in the carbon tetrachloride; or with the bromine solution alone; or in any desired manner, of which many are known in the art, to

render the vulcanized surface non-adherent to rubber deposited thereon from latex.

For the production of a series of replica samples, the process may be carried out as shown in Figs. 2 and 3. Accordingly, a layer 14 of latex composition is deposited on the upper surface 6 of the blanket 5 and the perforations 15 are blown therein by heating, and subsequent films are deposited and similarly perforated until the perforate rubber layer 16 is built up. Again, an impervious layer 17 of latex composition is deposited onto the upper surface of the layer 16 to bridge over and seal off the perforations 15, and is dried without being perforated. The replica blanket 13 may then be withdrawn from the blanket 5, as shown in Fig. 3, before or after application of a reinforcing ply, and may be vulcanized and treated as above described. In this manner as many identical blankets as may be desired can be produced either from the original blanket 5 or from any of the replica blankets 13.

While a particular method of producing the original blanket has been described, it may be produced upon an original perforate base instead of the air impermeable cavitated base employed in the method described. In this embodiment, a film of latex is spread in the ordinary manner to bridge the perforations, and a jet of fluid is forced through each perforation in the base to pierce the spread film. As the film is pierced to form perforations therein, the latex immediately surrounding the perforations may be set by heating if no coagulant is used, or by employing, as the jet of fluid, a coagulant for latex. The gelling or drying of the remainder of the pierced film may then be completed in any desired manner. A convenient method for carrying out this stage in the process is described in United States Letters Patent 2,032,923. After the desired number of superimposed perforate films have been produced in this way, the final sealing film or films are deposited thereon, as above described, that is, under conditions which gel or dry the final film or films but do not produce perforations therein. In this particular embodiment of the invention, heat may be employed to gel or dry the final layers without danger of expanding the air in the perforations therebelow, since that air in this case is not confined or entrapped.

The term "latex" as employed in this specification and the appended claims designates broadly coagulable dispersions of rubber or rubber-like materials as well as natural latex, which may be preserved or compounded or otherwise treated as desired, as by vulcanization, and which may be in normal, concentrated, diluted, or purified condition produced by methods well known in the art.

While certain present preferred methods of practicing the invention have been described, it may be understood that it may be otherwise practiced as will occur to those skilled in the art and within the spirit of the invention, and is to be limited only by the scope of the appended claims.

Having thus described my invention, what I claim and desire to protect by Letters Patent is:

1. The method of making a rubber sheet having cavities in the surface thereof which comprises depositing a film of latex composition onto a deposition blanket, concurrently drying or gelling said film and piercing said film with a plurality of fluid jets to form permanent perforations therein, depositing a film of latex onto said film and concurrently drying or gelling and 75 piercing said second named film, repeating said

operations until a perforate rubber sheet is built up, and thereafter depositing a sealing film of latex composition onto said perforate rubber sheet to bridge over and thereby seal exteriorly without filling up, an opening of each perforation, drying or gelling said sealing film so that it remains imperforate, and removing the cavitated, built-up blanket from the first-named deposition blanket.

2. A process for manufacturing a rubber sheet having cavities in the surface thereof which comprises spreading a coating of latex composition onto an air-impermeable deposition blanket having cavities or pits in the deposition surface thereof so as to entrap air between the latex coating and the backing in the said cavities or pits, and heating the backing to cause the entrapped air to expand and force its way through the latex coating while it is drying or gelling to form permanent perforations therein, depositing a film of latex onto said coating and concurrently drying or gelling and piercing said second named film, repeating said operations until a perforate rubber sheet is built up, and thereafter spreading a film of latex composition upon said perforate sheet to bridge over and thereby seal exteriorly, without filling up, an opening of each perforation, drying or gelling said film so that it remains imperforate, and removing the cavitated, built-up blanket from the first-named cavitated deposition blanket.

3. The method of making a rubber sheet having cavities in the surface thereof which comprises depositing a film of latex composition onto a deposition blanket, concurrently drying or gelling said film and piercing said film with a plurality of fluid jets to form permanent perfo-

rations therein, depositing a film of latex onto said film and concurrently drying or gelling and piercing said second named film, repeating said operations until a perforate rubber sheet is built up, and thereafter depositing a sealing film of latex composition onto said perforate rubber sheet to bridge over and thereby seal exteriorly, without filling up, an opening of each perforation, drying or gelling said sealing film so that it remains imperforate, removing the cavitated sheet from the blanket, and rendering the cavitated surface of said sheet non-adherent to an in situ solids deposit of a latex composition, substantially in the manner set forth.

10 15 20 25 30 35 4. The method of making a rubber sheet having cavities in the surface thereof which comprises the step of depositing a film of latex composition onto a deposition blanket, the step of concurrently drying or gelling said film and piercing said film with a plurality of fluid jets to form permanent perforations therein, the step of depositing a film of latex onto said film and concurrently drying or gelling and piercing said second named film, repeating said operations until a perforate rubber sheet is built up, and the step of depositing a sealing film of latex composition onto perforate rubber sheet to bridge over and thereby seal exteriorly, without filling up, an opening of each perforation, and the step of securing a ply of reinforcing material to said sealing layer, said steps being performed in the order named as a continuous series of operations while the built-up sheet remains in place upon the deposition blanket, and thereafter removing the reinforced cavitated sheet from said deposition blanket.

JAMES U. MANN.